

# UNITED STATES PATENT OFFICE.

NORBERT CEIPEK, OF VIENNA, AUSTRIA-HUNGARY.

## EXPLOSIVE COMPOUND.

No. 797,493.

Specification of Letters Patent.

Patented Aug. 15, 1905.

Application filed February 27, 1905. Serial No. 247,612.

*To all whom it may concern:*

Be it known that I, NORBERT CEIPEK, a subject of the Emperor of Austria-Hungary, residing at Vienna, Austria-Hungary, have invented certain new and useful Improvements in Explosive Compounds, of which the following is a specification.

Explosives are known which consist of ammonium nitrate and anilin nitrate. They possess high shattering effect and have little tendency to ignite combustible gases when they explode. Hence they are particularly applicable in fiery mines. By my invention explosives of this class are mixed with aluminium powder in order to enhance their shattering power.

The most advantageous mixture is from ten to fifteen parts of aluminium with from ninety to eighty-five parts of the ammonium nitrate

explosive, the latter being a mixture of eighty-five parts of ammonium nitrate with fifteen parts of anilin nitrate. The ingredients are mixed according to any known method.

I claim—

An explosive compound consisting of ten to fifteen parts by weight of aluminium combined with ninety to eighty-five parts by weight of a mixture formed of eighty-five per cent. of ammonium nitrate and fifteen per cent. of anilin nitrate.

In testimony whereof I have hereunto set my hand in presence of two subscribing witnesses.

NORBERT CEIPEK.

Witnesses:

JOSEF RUBASCH,  
ALVESTO S. HOGUE.